

Feb. 7, 1933.

F. F. FOWLE

1,896,613

## PROCESS OF TREATING ZINC COATED WIRE

Filed Aug. 13, 1931



Inventor  
*Frank F. Fowle,*

Schley & Trask

Attorneys

## UNITED STATES PATENT OFFICE

FRANK F. FOWLE, OF WINNETKA, ILLINOIS, ASSIGNOR TO INDIANA STEEL & WIRE COMPANY, OF MUNCIE, INDIANA, A CORPORATION OF INDIANA

## PROCESS OF TREATING ZINC-COATED WIRE

Application filed August 13, 1931. Serial No. 556,856.

It is the object of my invention to improve the quality of zinc-coated wire.

Zinc has the property of being toughened and densified by being worked mechanically 5 in a certain critical range of temperature. This range is from about 100° C. to about 150° C.; and within this temperature range it has malleability and ductility, and can be worked mechanically to advantage. At lower 10 and higher temperatures, it cannot be mechanically worked so advantageously, or with the same beneficial results.

My present invention takes advantage of this property of zinc. I heat the zinc-coated 15 wire to a temperature within the limits of this critical-temperature range, and then draw it through a die.

The accompanying drawing illustrates my invention. The single figure in said drawing 20 is a diagram showing an apparatus for carrying out my process.

The wire 10 to be treated, desirably a ferrous wire, has been suitably zinc-coated, as by the hot-galvanizing process. This zinc-coated wire 10, after being suitably heated to 25 a temperature within the aforesaid range where zinc has ductility and malleability, is supplied from any suitable source, such as a pay-out reel 11, to a wire-drawing die 12; through which it is drawn by the usual take-up block 13. The heating of the zinc-coated wire may be in any convenient way. The wire may be pre-heated in a furnace, and placed hot on the pay-out reel 11; in which 30 case it is desirable to have a suitable heat-retaining cover 14 over the pay-out reel and the roll of wire thereon. Instead, or in addition, a pre-heating furnace 15 may be located between the pay-out reel 11 and the die 12, and the wire passed through it to be heated to the desired temperature just before it reaches the die. The actual heating in either case may be to a temperature slightly 35 higher than the working temperature desired, to allow for a slight subsequent cooling before drawing.

The wire 10 has its zinc at a temperature within the critical range by the time it reaches the die 13. That die works the wire 40 as a whole, including the zinc of the coating,

with the result of toughening the zinc, densifying the zinc, and giving the whole wire a final accurate diameter.

I claim as my invention:—

1. The process of treating zinc-coated wire, which consists in drawing such wire through a die to reduce its diameter while it is at a temperature within the temperature range where zinc is improved in quality by mechanical working. 55

2. The process of treating zinc-coated wire, which consists in drawing such wire through a die to reduce its diameter while it is at a temperature between about 100° C. and about 150° C. 65

3. The process of treating zinc-coated ferrous wire, which consists in drawing such wire through a die to reduce its diameter while it is at a temperature within the temperature range where zinc is improved in 70 quality by mechanical working.

4. The process of treating zinc-coated ferrous wire, which consists in drawing such wire through a die to reduce its diameter while it is at a temperature between about 75 100° C. and about 150° C.

In witness whereof, I have hereunto set my hand at Indianapolis, Indiana, this 11th day of August, A. D. one thousand nine hundred and thirty-one. 80

FRANK F. FOWLE.